# EUROPEAN PATENT SPECIFICATION

(11) **EP 4 483 115 B1**
(45) Date of publication and mention of the grant of the patent: **08.07.2026**
(21) Application number: 23704186.8
(22) Date of filing: 15.02.2023
(51) Int. Cl.: F27D 1/00, C21D 9/56

(54) **HIGH PERFORMANCE THERMAL INSULATION OF A HEAT TREATMENT FURNACE FOR ANNEALING A CONTINUOUSLY MOVING STRIP**
HOCHLEISTUNGSWÄRMEDÄMMUNG EINES WÄRMEBEHANDLUNGSOFENS ZUM GLÜHEN EINES KONTINUIERLICH LAUFENDEN BANDES
ISOLATION THERMIQUE HAUTE PERFORMANCE D'UN FOUR DE TRAITEMENT THERMIQUE DE RECUIT D'UNE BANDE MOBILE EN CONTINU

(30) Priority: 21.02.2022 EP 22157736
(43) Date of publication of application: 01.01.2025
(73) Proprietor: John Cockerill SA, 4100 Seraing (BE)
(72) Inventor: PICARD, Paul-Henri, 4121 Neupré (BE)
(74) Representative: AWA Benelux
(86) International application number: PCT/EP2023/053691
(87) International publication number: WO 2023/156418

(56) References cited:
- EP-A1- 0 052 840
- CN-A- 109 341 353
- CN-U- 203 336 969
- US-A- 4 088 825
- US-A- 4 341 916
- US-A- 4 486 888
- US-A- 4 489 920

## Description

### Field of the Invention

The present invention relates to a specific insulation structure for lining furnaces such as a furnace in continuous bright annealing lines (BAL), which can be vertical or horizontal. More particularly, the insulation structure is intended to improve the thermal insulation performance of the annealing furnace and to ensure high quality of the steel.

The present invention is more generally applicable in technical field of continuous processing lines for strips of steel or aluminium, such as continuous annealing lines.

### Prior Art

It is known that bright annealing is an annealing process performed in a controlled atmosphere generally containing an inert gas and hydrogen. This controlled atmosphere reduces the surface oxidation to a minimum which results in a brighter surface mirror finish. As residual oxygen is entrained by the strip in the furnace, hydrogen should always be present in the furnace atmosphere, preferably with a content greater than 75%, the rest being inert gas such as nitrogen or argon. However in some annealing furnaces, hydrogen content can be lower than 75%.

In the vertical bright annealing furnace technology, the heating section of furnace is made in general of a stack of casing modules, comprising refractory bricks and an additional insulation. The traditional refractory bricks are often high purity bricks comprising 99% of alumina (Al₂O₃), made from bubble alumina, and typically with a bulk density of about 1800 kg/m³ and a porosity of 55%. The thermal conductivity of these traditional refractory bricks is typically 1.4 W/m°C at 1200°C, for a maximum service temperature of 1850°C. The additional insulation can be made from kaowool (ceramic) bulk fibres of silica and alumina, the composition of bulk fibres being for example of 53% of SiO₂ and 47% of Al₂O₃. A classic thickness of bricks / additional fibre insulation is comprised between 200 and 250mm.

Such a particular stack of casing modules is a proven technical solution comprising a lot of advantages, as the low maintenance and the facility to support scaffolding for this maintenance. Furthermore, it is easy to fix the heating elements thanks to embedded molybdenum anchors, and to provide protruding shield bricks to protect the heating elements. This is also a robust solution against strip breakage.

However, there are also some disadvantages, such as in particular a high thermal inertia which is the biggest issue, in particular with a high external casing temperature. Moreover, this solution is particularly heavy, with a large wall thickness (e.g. between 450 and 500mm) and a long time needed for erecting the walls of the furnace. Further brick supports are needed, being a source of large heat loss and thermal bridge. Another problem is that cracks can occur in the bricks, leading to pieces of brick and dust falling in the vertical furnace, possibly damaging the strip. These pieces of bricks and dust can also cause fire at the outlet of the furnace, owing to possible contact of very hot pieces with air containing hydrogen at this location.

Solutions not involving ceramic bricks assemblies anymore are known. For example, Unifrax LLC (Tonawanda NY 14150, USA) has provided furnace lining (temperatures up to 1300°C) under the form of polycrystalline fibre modules (Saffil^{®} M-Fil Anchor-Loc^{®} Modules), for example in forging applications.

Document US 2005/055940 A1 discloses a lining for a furnace, the lining having insulating material attached to an inside wall of the furnace, the insulating material in use having a hot face which faces inwardly of the furnace and a cold face at or adjacent the furnace wall, wherein a protective element is provided at least partially to cover the hot face, the protective element being secured relative to the hot face by a securing means which co-operates with a member which is embedded in the insulating material, and wherein the securing means is adapted to engage the member after the member is embedded in the insulating material. The furnace lining includes a plurality of individual blocks or modules of insulating material, each attached at the inside wall of the furnace, each module including a ceramic blanket which is folded to a block-like shape with the folds extending transversely to the furnace wall.

The protective element is made at least substantially of one or more of a ceramic material, a blanket of silica free insulation, a high-temperature resistant textile material, and a higher temperature resistant high alumina insulation than other insulation material of the lining.

Is also disclosed a fixing attached by one or more fasteners to the furnace wall made of a steel panel, the fixing having a hooked part which is embedded in the fibres of the module in a position where fixing rods (or tubes) are inserted through the folds to co-operate with the hooked part. The rods may co-operate with a plurality of fixings attaching modules to the inside of the furnace wall.

Utility model CN203336969U relates to an all-fiber energy-saving furnace lining outer cover. The all-fiber energy-saving furnace lining outer cover comprises a furnace body steel casing, polycrystalline mullite composite fiber bricks, an aluminum silicate zirconium fiberboard, supporting strip bricks, electric heating elements, polycrystalline mullite composite fiber lower surrounding bricks and polycrystalline mullite composite fiber upper surrounding bricks, wherein the polycrystalline mullite composite fiber bricks, the aluminum silicate zirconium fiberboard, the supporting strip bricks, the electric heating elements, the polycrystalline mullite composite fiber lower surrounding bricks and the polycrystalline mullite composite fiber upper surrounding bricks are arranged in the furnace body steel casing. The electric heating elements are arranged on the supporting strip bricks, the aluminum silicate zirconium fiberboard is arranged between the furnace body steel casing and the polycrystalline mullite composite fiber bricks, a zirconium fiber assembly is arranged at the top of a furnace lining, and the inner surface of the furnace lining is provided with an infrared radiation porous ceramic layer.

Document US4486888A discloses a furnace including a jacket which is removably mounted to a bottom plate construction so that the jacket can be mounted on anyone of a number of the bottom plate constructions. A cap is removably secured on an upper part of the jacket by latches, and electric resistance elements are mounted adjacent to an inner surface of the jacket by a plurality of strips having pins thereon. Since the jacket is removably mounted on the bottom plate construction, after a burning process has been completed, the jacket can be removed from the bottom plate construction and placed on another similar bottom plate construction to initiate another burning process while the products which have been previously burned are allowed to cool. In the event that quick cooling of the products is not desirable, the cap may be removed and replaced by a simple, intermediate cap so that the products are allowed to cool more slowly.

### Aims of the Invention

The present invention aims to provide an insulated wall structure for e.g. a vertical bright annealing furnace which does not present the drawbacks of the above-mentioned prior art structures, and which optimizes both thermal insulation performances and thermal inertia, while ensuring high quality of the thermally-treated steel strip.

The aimed low thermal inertia of the structure of the present invention should provide a more flexible furnace temperature with a shorter response time, allowing to recover expected operating conditions more quickly and the possibility to quickly switch off the furnace if necessary.

The invention also aims to provide an innovative solution, having elements which are light and fast to erect. The structure of the present invention should allow to avoid the risk of cracks related to the use of insulating bricks, and of pieces of bricks and dust falling in the vertical furnace and thus minimize possible damage on the strip when it is travelling.

Further the present invention aims at replacing the insulating bricks in their role of mechanical support of the heating elements, also considering that the new support should not react with the hydrogen atmosphere in the furnace.

Finally the invention should render not necessary to have brick support at the base of the furnace, avoiding thermal bridges.

### Summary of the Invention

A first aspect of the present invention relates to a furnace for performing a thermal treatment of a continuously moving metal strip, preferably under hydrogen protective atmosphere, having :
- a hybrid wall lining facing inwardly of the furnace, wherein said hybrid wall lining comprises a stack of polycrystalline fibre modules, and graphite lintels being fixed between or in said modules, and
- electric heating elements provided inside the furnace along one or more vertical walls and fixed on the side of the hybrid wall lining facing inwardly of the furnace,

wherein said polycrystalline fibre modules comprise fibres with at least 95% of Al₂O₃, and preferably at least 97% of Al₂O₃, so as to be compatible with a hydrogen protective atmosphere, the thickness of the polycrystalline fibre modules being comprised between 200 and 500mm,
wherein the electric heating elements are attached to the graphite lintels thanks to a first anchoring system, and
wherein the graphite lintels are suitable to protect the heating elements against strip deviations, by being cantilevered above the heating elements and protruding from the wall lining inside the furnace.

According to preferred embodiments of the invention, the furnace is further limited by one of the following features or by a suitable combination thereof :
- each of the polycrystalline fibre modules is provided with a second anchoring system suitable to fix said module to at least one adjacent module and/or to the external casing of the furnace ;
- said wall lining comprises additional bulk fibre or fibre blanket or board between the stack of polycrystalline modules and the external casing of the furnace ;
- the additional bulk fibre or fibre blanket or board has a thickness between 20 and 250mm ;
- supporting tubes are, at one end, attached inside the graphite lintels and, at the other end, welded, perpendicularly, to the casing of the furnace in order to support the graphite lintels ;
- a space is provided between the interior end of each graphite lintel and the casing of the furnace, said space comprising the tube supporting the lintel and being filled with bulk fibres ;
- the heating elements are forming a continuous planar serpentine and the graphite lintels are arranged in horizontal rows and are provided with the first anchoring system made of vertical hooks, so that adjacent vertical hooks located in two vertically adjacent lintel rows are respectively supporting the lower and upper successive loops of the heating element ;
- the furnace is a furnace in a continuous annealing line ;
- the furnace is a vertical furnace ;
- the furnace is a horizontal furnace.

A second aspect of the present invention relates to the use of the furnace described above, for performing a thermal treatment of a continuously moving metal strip, preferably under a controlled hydrogen protective atmosphere.

Preferably, the controlled hydrogen protective atmosphere has a hydrogen content greater than 75%, the rest being inert gas.

Advantageously, the thermal treatment of a continuously moving metal strip is a treatment for strips of steel or aluminium, preferably in continuous annealing lines.

### Brief Description of the Drawings

Figure 1 represents a cross-sectional longitudinal view of a vertical bright annealing furnace of prior art.
Figure 2 represents a cross-sectional lateral view of a vertical bright annealing furnace of prior art.
Figure 3 represents a 3D view of a part of a furnace with a lining comprising polycrystalline fibre modules according to the present invention.
Figure 4 represents a first cross-sectional view of the furnace of Figure 3.
Figure 5 represents a second cross-sectional view of the furnace of Figure 3.
Figure 6 represents a third cross-sectional view of the furnace of Figure 3.
Figure 7 represents a detailed cross-sectional view of an anchoring system of a heating element in a common vertical bright annealing furnace of prior art.
Figure 8 represents a detailed cross-sectional view of an anchoring system of a heating element in a module of a vertical bright annealing furnace according to the present invention.
Figure 9 shows the temperature distribution in the thickness of a wall of a vertical bright annealing furnace of prior art.
Figure 10 shows the temperature distribution in the thickness of a wall of a bright annealing furnace with a lining comprising polycrystalline fibre modules according to the present invention.
Figure 11 represents a detailed view of a system for anchoring the polycrystalline fibre modules to the furnace casing according to prior art.
Figure 12 represents a detailed cross-sectional view of an anchoring system of a heating element in a module of a vertical bright annealing furnace according to the present invention, in which the polycrystalline fibre modules have been replaced by graphite rigid felt boards.

### Description of Preferred Embodiments of the Invention

The present invention relates to a new wall structure 2 for a vertical bright annealing furnace 1. This specific structure comprises a stack of insulating polycrystalline fibre modules 3 as illustrated by Figures 3 to 6. Once the modules 3 are assembled and fixed to form the wall 2, an additional fibre blanket 4 can be added in the furnace 1 between the polycrystalline fibre modules 3 and the casing.

Each module 3 has preferably a thickness between 400 and 500 mm, and more preferably of 450 mm. The additional fibre blanket 4 has preferably a thickness between 20 and 50mm, and more preferably of 25 mm.

The insulating polycrystalline fibre modules 3 preferably comprise fibre with at least 95-97% of Al₂O₃.

As explained below, and illustrated by Figures 3-4, 6 and 8, electric heating elements 6 are provided inside the furnace 1. The heating elements 6 are fixed to the modules 3 by an anchoring system 5. In order to protect the heating elements 6 against shocks due to the contact with the running or broken strip in the furnace 2, graphite lintels 11 are provided, preferably provided with chicanes. Graphite lintels 11 are fixed in the wall 2 between and/or within modules 3, and are cantilevered just above each heating element 6 (see Figures 6 and 8). This is more detailed in the following sections of the description.

The wall 2 obtained with the modules 3 of the present invention exhibits an improved thermal insulation and thermal inertia offering a more flexible furnace temperature. This new solution will give the opportunity to have a wall lighter and easier to build, with no risk of cracks or fire in operation.

### Polycrystalline fibre modules

Polycrystalline fibre modules 3 of the present invention can be for example a polycrystalline Saffil^{®} M-Fil prefabricated modules (source: Unifrax documentation). Saffil^{®} M-Fil modules 3 are manufactured from polycrystalline wool into a standard edge-stacked construction format. The modules are made of fibre compressed with cardboard (ou wooden) side plates with banding straps. These prefabricated modules 3 are specifically designed to meet the thermal insulation requirements of industrial furnaces. As illustrated in Figure 11, Saffil modules can be produced with various anchoring systems 14, 16, known per se of the skilled person and often commercially available, to enable quick, easy and efficient installation for most lining applications.

### Graphite rigid felt boards

In an alternative embodiment shown on Figure 12, polycrystalline alumina fibre modules can be replaced by a stack of graphite rigid felt boards 7, preferably horizontally arranged. This material has a carbon content of 99.5% and is very light (bulk density of about 0.2 g/cm³).

### Polycrystalline fibre modules and heating elements : assembly and anchoring method

Polycrystalline fibre modules 3 according to the present invention can be assembled and fixed according different fixing methods known from prior art (see for example Unifrax documentation).

A first system, named *"RX2 anchoring system"* is a patented metal support in 321 stainless steel, which provides rapid attachment of the module 3 to the furnace casing via the external side fastener which is screwed onto a pre-welded stud. Rail, washer, nut, stud and ceramic arc shield are supplied (see US 2005/055940 A1, ref. 14, 15, 18).

A second system, named *"Thread Lock (TL) anchoring system" 14* and illustrated in Figure 11, is attached to the furnace casing 15 by a central anchor in 304 stainless steel. Threaded studs 16 are pre-welded on the internal side of the furnace casing and the module anchor 14 is screwed on the stud by using a tool 20 such as a ratchet drive. The module anchor 14 has two wings terminated each with a hole 17 for supporting an assembly tube or rod linked in the same manner to adjacent module anchors.

*The "TL anchoring system"* has been especially designed for three reasons:
- as a complementary assembly system to RX2 or similar ;
- for the lining of small furnaces ;
- to repair all types of lining installations.

Other similar systems are available off the shelf.

### Heating Element Protection

In the bright annealing vertical furnace technology of prior art, as illustrated in Figure 7, shield bricks 10 containing 99% Al₂O₃ are provided to protect the heating elements 6. These shield bricks are easy to implement, because they are refractory bricks 8 being placed so that they protrude inside the furnace 1, just above the vertical heating elements 6. In this manner, the travelling strip is prevented to hit the heating elements 6 being below the shield bricks 10.

In the case of the present invention, the fibre modules 3 per se do not allow to protect the heating elements 6 while forming the walls 2 of the furnace 1. Another shielding solution is therefore needed.

As illustrated in Figures 6 and 8, according to the present invention, graphite lintels 11 have been provided between fibre modules 3, just above the heating elements 6.

Graphite lintels 11 can be advantageously obtained from machinable extruded graphite. Graphite is dense, has high temperature resistance and does not react with hydrogen. See example of data sheet below (mechanical data : "with the grain") :

| | | |
|---|---|---|
| Bulk density | g/cm³ | 1.7 |
| Open porosity | % | 17 |
| Young modulus | GPa | 10 |
| Flexural strength | MPa | 18 |
| Compressive strength | MPa | 39 |
| Tensile strength | Mpa | 13 |

In a vertical furnace or in a horizontal furnace with heating elements arranged along vertical walls, the graphite lintels 11 advantageously protrude from a vertical wall line inside the furnace 1 to protect the heating elements 6. Additionally, the graphite lintels 11 have also the function of supporting and guiding the heating elements 6, via an anchoring system 5, for example under the form of molybdenum hooks.

The heating elements 6 are preferably electric heating elements arranged according to a planar serpentine connected at each of its two ends to an insulated connector 30 going through the wall lining 2 and the external casing 15 of the furnace 1 to the power supply.

The graphite lintels 11 are arranged in horizontal rows and are provided with anchoring system 5 made of vertical hooks, preferably made of molybdenum, so that adjacent vertical hooks located in two vertically adjacent lintel rows are respectively supporting the lower and upper successive loops of the heating element.

Still according to the invention (see Figure 8), supporting tubes 12 are welded to the casing 15 of the furnace in order to support the graphite lintels 11 in the insulation assembly. Further, a space 13 is provided between the back of the lintel 11 and the casing 15 of the furnace. This space 13 encloses the tube 12 supporting the lintel 11, and can be filled with bulk fibres known *per* se of the skilled person. In case the wall lining 2 comprises boards of graphite rigid felt, said boards are supported by the horizontal layers of graphite lintels 11 and attached to the casing with usual anchoring means (such as for bricks).

Such as polycrystalline alumina fibre modules, graphite lintels 11 do not have the defects of the shield bricks 10 of prior art, such as cracks or breaks prone to occur in the bricks, possibly leading to pieces of brick and dust falling in the vertical furnace, and possibly damaging the strip or causing fire at the outlet of the furnace.

In a horizontal furnace, two configurations can be adopted :
- in a first configuration, the heating elements are located in the vertical walls of the furnace. To take over the protection role of the insulation bricks against the deviation of the strip, the insulation fibre structure should be provided with a protective frame with at least two vertical lintels and two horizontal lintels, as described above, for each heating unit (not shown) ;
- in a second configuration, the heating elements are provided in the dome of the furnace. In this case, there is no (or less) need for protecting the heating elements.

### Performances

The performances of the polycrystalline fibre modules 3 of the present invention are compared to the stack of casing modules of prior art, comprising refractory bricks and additional insulation. The results are illustrated in Figure 9 representing the temperature distribution in the thickness of a wall of the vertical bright annealing furnace of prior art, and in Figure 10 representing the temperature distribution in the thickness of a wall of the bright annealing furnace with the structure of the present invention.

The calculation hypotheses are the same for both cases.

In the example, the wall of the bright annealing furnace of prior art comprises stack of casing modules with refractory bricks 8 and additional insulation 9 (made of bulk fibres). The wall of a bright annealing furnace according to the present invention comprises a structure with polycrystalline fibre modules 3 having a thickness of 450 mm and an additional fibre blanket (backup layer faced with aluminium foil, e.g. Insulfrax^{®} S blanket, documentation Unifrax) having a thickness of 25 mm.

As illustrated by Figure 9, in case of the furnace of prior art, the external casing temperature of the furnace is 132°C, leading to a thermal flux of 1460 W/m2.

As illustrated by Figure 10, in case of the furnace of the present invention, the external casing temperature of the furnace is 115°C, leading to a thermal flux of 1122 W/m2.

The lining of the furnace walls in the present invention allows a reduction of external casing temperature of 17°C and of thermal flux of 23%.

### Reference Symbols

- 1: Vertical bright annealing furnace
- 2: Wall of the furnace (with lining)
- 3: Polycrystalline fibre modules
- 4: Additional fibre blanket
- 5: Anchoring system of a heating element
- 6: Heating element
- 7: Graphite rigid felt board
- 8: Refractory brick
- 9: Additional insulation
- 10: Shield brick
- 11: Graphite lintel
- 12: Supporting tube
- 13: Space between the lintel and the furnace casing
- 14: "Thread Lock" anchoring system of the module
- 15: Furnace casing
- 16: Threaded stud
- 17: Tube supporting wing
- 18: Flange hex nut
- 19: Sliding collar
- 20: Tool
- 30: Insulated connector

## Claims

1. A furnace (1) for performing a thermal treatment of a continuously moving metal strip, preferably under hydrogen protective atmosphere, having :
- a hybrid wall lining (2) facing inwardly of the furnace (1), wherein said hybrid wall lining (2) comprises a stack of polycrystalline fibre modules (3), and graphite lintels (11) being fixed between or in said modules (3), and
- electric heating elements (6) provided inside the furnace (1) along one or more vertical walls and fixed on the side of the hybrid wall lining (2) facing inwardly of the furnace (1),
wherein said polycrystalline fibre modules (3) comprise fibres with at least 95% of Al₂O₃, and preferably at least 97% of Al₂O₃, so as to be compatible with a hydrogen protective atmosphere, the thickness of the polycrystalline fibre modules (3) being comprised between 200 and 500mm, and
wherein the electric heating elements (6) are attached to the graphite lintels (11) thanks to a first anchoring system (5),
and wherein the graphite lintels (11) are suitable to protect the heating elements (6) against strip deviations, by being cantilevered above the heating elements (6) and protruding from the wall lining (2) inside the furnace (1).

2. The furnace (1) according to claim 1, wherein each of the polycrystalline fibre modules (3) is provided with a second anchoring system (14, 16) suitable to fix said module (3) to at least one adjacent module (3) and/or to the external casing (15) of the furnace.

3. The furnace (1) according to claim 1 or 2, wherein said wall lining (2) comprises additional bulk fibre or fibre blanket or board (4) between the stack of polycrystalline modules (3) and the external casing (15) of the furnace (1).

4. The furnace (1) according to claim 3, wherein the additional bulk fibre or fibre blanket or board (4) has a thickness between 20 and 250mm.

5. The furnace (1) according to claim 1, wherein supporting tubes (12) are, at one end, attached inside the graphite lintels (11) and, at the other end, welded, perpendicularly, to the casing (15) of the furnace (1) in order to support the graphite lintels (11).

6. The furnace (1) according to claim 5, wherein a space (13) is provided between the interior end of each graphite lintel (11) and the casing (15) of the furnace (1), said space (13) comprising the tube (12) supporting the lintel (11) and being filled with bulk fibres.

7. The furnace (1) according to claim 1, wherein the heating elements (6) are forming a continuous planar serpentine and wherein the graphite lintels (1) are arranged in horizontal rows and are provided with the first anchoring system (5) made of vertical hooks, so that adjacent vertical hooks located in two vertically adjacent lintel rows are respectively supporting the lower and upper successive loops of the heating elements (6).

8. The furnace (1) according to anyone of the preceding claims, wherein the furnace is a furnace in a continuous annealing line.

9. The furnace (1) according to anyone of the preceding claims, wherein the furnace (1) is a vertical furnace.

10. The furnace (1) according to anyone of claims 1 to 8, wherein the furnace (1) is a horizontal furnace.

11. Use of the furnace according to anyone of the preceding claims, for performing a thermal treatment of a continuously moving metal strip, preferably under a controlled hydrogen protective atmosphere.

12. Use according to claim 11, wherein the controlled hydrogen protective atmosphere has a hydrogen content greater than 75%, the rest being inert gas.

13. Use according to claim 11, wherein the thermal treatment of a continuously moving metal strip is a treatment for strips of steel or aluminium, preferably in continuous annealing lines.

## Patentansprüche

1. Ofen (1) zum Durchführen einer Wärmebehandlung eines kontinuierlich bewegten Metallbands, vorzugsweise unter Wasserstoff-Schutzatmosphäre, der Folgendes aufweist:
- eine hybride Wandverkleidung (2), die der Innenseite des Ofens (1) zugewandt ist, wobei die hybride Wandverkleidung (2) einen Stapel aus polykristallinen Fasermodulen (3) und Graphitstürze (11), die zwischen oder in den Modulen (3) befestigt sind, umfasst, und
- elektrische Heizelemente (6), die im Inneren des Ofens (1) entlang einer oder mehrerer vertikaler Wände bereitgestellt und an der hybriden Wandverkleidung (2), die der Innenseite des Ofens (1) zugewandt ist, befestigt sind,
wobei die polykristallinen Fasermodule (3) Fasern mit mindestens 95 % Al₂O₃, vorzugsweise mindestens 97 % Al₂O₃, umfassen, um mit einer Wasserstoff-Schutzatmosphäre kompatibel zu sein, wobei die Stärke der polykristallinen Fasermodule (3) zwischen 200 und 500 mm liegt, und
wobei die elektrischen Heizelemente (6) mittels eines ersten Verankerungssystems (5) an den Graphitstürzen (11) befestigt sind,
und wobei die Graphitstürze (11) geeignet sind, die Heizelemente (6) gegen Bandabweichungen zu schützen, indem sie auskragend über den Heizelementen (6) sind und von der Wandverkleidung (2) in das Innere des Ofens (1) hervorstehen.

2. Ofen (1) nach Anspruch 1, wobei jedes der polykristallinen Fasermodule (3) mit einem zweiten Verankerungssystem (14, 16) versehen ist, das geeignet ist, um das Modul (3) an mindestens einem angrenzenden Modul (3) und/oder an dem Außengehäuse (15) des Ofens zu befestigen.

3. Ofen (1) nach Anspruch 1 oder 2, wobei die Wandverkleidung (2) zusätzlich lose Fasern oder Faserfilz oder Faserplatten (4) zwischen dem Stapel der polykristallinen Module (3) und dem Außengehäuse (15) des Ofens (1) umfasst.

4. Ofen (1) nach Anspruch 3, wobei die zusätzlichen losen Fasern oder der Faserfilz oder die Faserplatte (4) eine Stärke zwischen 20 und 250 mm aufweisen.

5. Ofen (1) nach Anspruch 1, wobei Stützrohre (12) an einem Ende im Inneren der Graphitstürze (11) angebracht sind und an dem anderen Ende senkrecht an das Gehäuse (15) des Ofens (1) angeschweißt sind, um die Graphitstürze (11) zu tragen.

6. Ofen (1) nach Anspruch 5, wobei zwischen dem inneren Ende von jedem Graphitsturz (11) und dem Gehäuse (15) des Ofens (1) ein Raum (13) bereitgestellt ist, wobei der Raum (13) das Rohr (12) zum Tragen des Sturzes (11) umfasst und mit losen Fasern gefüllt ist.

7. Ofen (1) nach Anspruch 1, wobei die Heizelemente (6) eine durchgehende ebene Schlange bilden und wobei die Graphitstürze (11) in horizontalen Reihen angeordnet sind und mit dem ersten Verankerungssystem (5) aus vertikalen Haken versehen sind, sodass benachbarte vertikale Haken, die sich in zwei vertikal angrenzenden Sturzreihen befinden, jeweils die untere und die obere aufeinanderfolgenden Schleife der Heizelemente (6) tragen.

8. Ofen (1) nach einem der vorherigen Ansprüche, wobei der Ofen ein Ofen in einer kontinuierlichen Glühlinie ist.

9. Ofen (1) nach einem der vorherigen Ansprüche, wobei der Ofen (1) ein Vertikalofen ist.

10. Ofen (1) nach einem der Ansprüche 1 bis 8, wobei der Ofen (1) ein Horizontalofen ist.

11. Verwendung des Ofens nach einem der vorherigen Ansprüche zum Durchführen einer Wärmebehandlung eines kontinuierlich bewegten Metallbands, vorzugsweise unter einer kontrollierten Wasserstoff-Schutzatmosphäre.

12. Verwendung nach Anspruch 11, wobei die kontrollierte Wasserstoff-Schutzatmosphäre einen Wasserstoffgehalt von mehr als 75 % aufweist, wobei der Rest ein Inertgas ist.

13. Verwendung nach Anspruch 11, wobei die Wärmebehandlung eines kontinuierlich bewegten Metallbands eine Behandlung für Bänder aus Stahl oder Aluminium ist, vorzugsweise in kontinuierlichen Glühlinien.

## Revendications

1. Four (1) destiné à effectuer un traitement thermique d'une bande métallique qui se déplace en continu, de préférence sous atmosphère protectrice d'hydrogène, ayant :
- un revêtement de paroi hybride (2) qui fait face à l'intérieur du four (1), dans lequel ledit revêtement de paroi hybride (2) comprend un empilement de modules de fibres polycristallines (3), et des linteaux en graphite (11) fixés entre ou dans lesdits modules (3), et
- des éléments chauffants électriques (6) prévus à l'intérieur du four (1) le long d'une ou plusieurs parois verticales et fixés sur le côté du revêtement de paroi hybride (2) qui fait face à l'intérieur du four (1),
dans lequel lesdits modules de fibres polycristallines (3) comprennent des fibres contenant au moins 95 % d' Al₂O₃, et de préférence au moins 97 % d' Al₂O₃, de manière à être compatibles avec une atmosphère protectrice d'hydrogène, l'épaisseur des modules de fibres polycristallines (3) étant comprise entre 200 et 500 mm, et
dans lequel les éléments chauffants électriques (6) sont fixés sur les linteaux en graphite (11) grâce à un premier système d'ancrage (5),
et dans lequel les linteaux en graphite (11) sont adaptés pour protéger les éléments chauffants (6) contre les écarts de la bande, en étant en porte-à-faux au-dessus des éléments chauffants (6) et en faisant saillie depuis le revêtement de paroi (2) à l'intérieur du four (1).

2. Four (1) selon la revendication 1, dans lequel chacun des modules de fibres polycristallines (3) est équipé d'un deuxième système d'ancrage (14, 16) adapté pour fixer ledit module (3) sur au moins un module adjacent (3) et/ou sur l'enceinte externe (15) du four.

3. Four (1) selon la revendication 1 ou 2, dans lequel ledit revêtement de paroi (2) comprend des fibres en bourre ou un tissu en fibres ou un panneau de fibres (4) supplémentaire(s) entre l'empilement de modules de fibres polycristallines (3) et l'enceinte externe (15) du four (1).

4. Four (1) selon la revendication 3, dans lequel les fibres en bourre ou le tissu en fibres ou le panneau de fibres (4) supplémentaire(s) présente(nt) une épaisseur comprise entre 20 et 250 mm.

5. Four (1) selon la revendication 1, dans lequel des tubes de support (12) sont, à une extrémité, fixés à l'intérieur des linteaux en graphite (11) et, à l'autre extrémité, soudés perpendiculairement à l'enceinte (15) du four (1) afin de supporter les linteaux en graphite (11).

6. Four (1) selon la revendication 5, dans lequel un espace (13) est prévu entre l'extrémité intérieure de chaque linteau en graphite (11) et l'enceinte (15) du four (1), ledit espace (13) comprenant le tube (12) qui supporte le linteau (11) et étant rempli de fibres en bourre.

7. Four (1) selon la revendication 1, dans lequel les éléments chauffants (6) forment un serpentin plat continu et dans lequel les linteaux en graphite (11) sont disposés en rangées horizontales et sont équipés du premier système d'ancrage (5) constitué de crochets verticaux, de sorte que les crochets verticaux adjacents situés sur deux rangées de linteaux verticalement adjacentes supportent respectivement les boucles inférieures et supérieures successives des éléments chauffants (6).

8. Four (1) selon l'une quelconque des revendications précédentes, dans lequel le four est un four d'une ligne de recuit continu.

9. Four (1) selon l'une quelconque des revendications précédentes, dans lequel le four (1) est un four vertical.

10. Four (1) selon l'une quelconque des revendications 1 à 8, dans lequel le four (1) est un four horizontal.

11. Utilisation du four selon l'une quelconque des revendications précédentes, pour effectuer un traitement thermique d'une bande métallique qui se déplace en continu, de préférence sous une atmosphère protectrice d'hydrogène contrôlée.

12. Utilisation selon la revendication 11, dans laquelle l'atmosphère protectrice d'hydrogène contrôlée présente une teneur en hydrogène supérieure à 75 %, le reste étant un gaz inerte.

13. Utilisation selon la revendication 11, dans laquelle le traitement thermique d'une bande métallique qui se déplace en continu est un traitement pour des bandes d'acier ou d'aluminium, de préférence sur des lignes de recuit continu.
